

## UNITED STATES PATENT OFFICE.

ROBERT ZIMMERMANN, OF TUBACH, SWITZERLAND, ASSIGNOR TO FIRM OF TEXTIL-WERK HORN A.G., OF HORN AM BODENSEE, SWITZERLAND.

PROCESS FOR THE MANUFACTURE OF A CELLULOSE COMPOUND INDIFFERENT TO SUBSTANTIVE COLORS.

No Drawing.

Application filed March 28, 1923. Serial No. 628,323.

To all whom it may concern:

Be it known that I, ROBERT ZIMMERMANN, a citizen of the Republic of Switzerland, residing at Tubach, Canton St. Gall, Switzerland, have invented certain new and useful Improvements in Processes for the Manufacture of a Cellulose Compound Indifferent to Substantive Colors, of which the following is a specification.

10 It is known to produce effect-threads in cotton or other vegetable fibres by causing acid chlorides of the aromatic series to act in the presence of indifferent solvents on vegetable fibres previously treated with alkalis. This process has however the drawback of being relatively expensive owing to the acid chlorides utilized.

20 This invention relates to a process for rendering vegetable fibres indifferent to substantive colors or dyes, according to which vegetable fibres rendered alkaline in the well known manner, are treated with aromatic sulpho-chlorides, more particularly with para-toluol-sulphochloride in suitable solvents and at suitable temperatures. This process has the advantage that cheap materials may be used for carrying out the process and that the effect is better than in the above stated known process.

30 The alkalinized cellulose fibre insoluble in alkali and water is converted according to this process into an ester compound which can no longer be dyed in a hot soap bath with substantive colors.

35 In the case of the transformation (immunization) of yarn, the process may be as follows:

40 By heating industrial alcohol containing water, for instance 95% alcohol, with pieces of soda in excess, there is prepared in a well known manner first as strong an alcoholic solution of soda as possible, for instance of 14%, which on being cooled forms a brownish liquid. If carefully bleached 45 cotton, as free from fat as possible, either loose or in the form of yarn or fabric is immersed in the said solution and left for several hours, the said cotton will be converted in the well known manner into its 50 soda compound, that is to say alkalinized. The cotton is thereupon withdrawn and the lye adhering to it, removed by pressure or centrifugal action.

1 kg. of the alkalinized and centrifuged 55 yarn is immersed in 15 litres of a tetrachloride of carbon of 15-20°—using a clay or enamelled vessel—which contains 200 gr. para-toluol-sulphochloride per litre. After a short time a reaction takes place 60 with a rise of temperature which however does not reach the boiling point of the liquid. Care must be taken that the yarn always remains under the surface of the liquid. The whole is then allowed to cool 65 for several hours, and heated again by supplying heat by external means until the boiling point is nearly reached. The yarn is then withdrawn and pressed out, and afterwards all sulpho-chloride and solvent 70 are removed from it by passing it several times through a soap solution of 60° C. and rinsing until it is quite odorless. A yellowish-white end product thereupon is obtained by means of a hot soda washing 75 and by the usual chlorine bleaching with acids and washing out, the said end product being centrifuged and dried. The immune yarn thus obtained has been somewhat shortened owing to the esterification, but at the same time its weight has been increased 80 to a considerable extent which may amount to 20% and more. When dyeing with substantive colors in hot soda-soap solution, the said yarn proves to be indifferent. Unlike the ordinary yarn, its strength is un- 85 affected by the usual bleaching chlorine solution, even if exposed to its action cold for several days. It also resists diluted acids much better and its indifference to substantive colors remains unaffected even 90 by the acid used for obtaining a transparent effect and by the mercerizing lye provided that it is treated cold and for a short time and rinsed immediately afterwards, but it shows a not inconsiderable fixing property 95 as regards basic colors.

By weaving it together with raw or bleached cotton yarn, it may be used advantageously for the manufacture of colored pattern fabrics and transparent fabrics. 100

Yarn previously treated with vat dyes, for instance with "indanthrene" blue, can in the same way be rendered immune to substantive colors. By weaving such immune 105 colored yarn with the ordinary yarn and subsequently dyeing with substantive colors,

textile fabrics can be prepared with patterns in several colors of the most varied kinds.

In the process of preparation, the treatment with alkali may also be carried out with potassium hydroxide, and instead of carbon tetra-chloride there may also be used a sulpho-chloride solvent or other chlorinated hydrocarbons of the fatty series, also hydrocarbons of the petroleum series and benzol and its homologues. It is also possible to prepare immune cellulose products with other sulpho-chlorides of the non-substituted and substituted aromatic hydrocarbons, for instance with benzo-sulpho-chloride, ortho-toluol-sulpho-chloride, xylol- and naphthaline-sulphochlorides and with chlorine, bromine and nitro-derivates of all these compounds.

I claim:

- 20 1. Process for converting alkalized cellulose fibres into a fibre which can no longer be dyed with substantive colors which process comprises treating the alkalized cellulose with aromatic sulpho-chlorides.
- 25 2. Process for the manufacture of a cellulose fibre indifferent to substantive colors which process comprises subjecting the cellulose fibre to a treatment with an alcoholic solution of caustic soda, and treating the

alkalized cellulose with aromatic sulpho-chlorides.

3. Process for the manufacture of a cellulose fibre indifferent to substantive colors which process comprises subjecting the cellulose fibre to an alkalizing treatment, and 35 treating the alkalized cellulose with para-toluol-sulpho-chloride.

4. Process for rendering vegetable fibres immune to substantive dyes, which comprises treating the fibre with alkali and then 40 subjecting the fibre to the action of a solution of aromatic sulpho-chloride in carbon tetra-chloride and washing the fibre.

5. Process for rendering vegetable fibres immune to substantive dyes, which comprises treating fibre with alkali and then 45 subjecting the fibre to the action of a solution of para-toluol-sulpho-chloride in carbon tetra-chloride.

6. Process for the manufacture of a cellulose fibre indifferent to substantive colors, which process comprises treating the fibre with vat-dyes, subjecting this fibre to an alkalizing treatment and treating the alkalized fibre with aromatic sulpho-chlorides. 50 55

In testimony whereof I affix my signature.

ROBERT ZIMMERMANN.